# EUROPEAN PATENT SPECIFICATION

(11) **EP 2 679 691 B1**
(45) Date of publication and mention of the grant of the patent: **17.04.2019**
(21) Application number: 13171750.6
(22) Date of filing: 12.06.2013
(51) Int. Cl.: C21C 5/00, C21C 5/28, C22B 3/00, C22B 3/04, C22B 3/20, C22B 23/00, C22C 1/00, C22C 33/04, C22C 38/40

(54) **Method for manufacturing an austenitic stainless steel from a nickel laterite ore and a chromite ore**
Verfahren zur Herstellung eines austenitischen rostfreien Stahls aus einer von Nickel-Laterit-Erz und einem Chromeisenerz
Procédé de fabrication d'un acier inoxydable austénitique à partir d'un minerai de latérite de nickel et de chromite

(30) Priority: 28.06.2012 TW 101123242
(43) Date of publication of application: 01.01.2014
(73) Proprietor: Yieh United Steel Corp., Kaohsiung Hsien (TW)
(72) Inventor: HSU, Wen-Chien, 81150 Kaohsiung City (TW); HUANG, Pei-Te, 833 Kaohsiung City (TW); WU, Yi-Cheng, 813 Kaohsiung City (TW); YANG, Cheng-Tung, 820 Kaohsiung City (TW)
(74) Representative: Carpmael, Robert Maurice Charles

(56) References cited:
- WO-A2-01/86006
- DE-A1-102007 050 478
- FR-A5- 2 121 165
- US-A- 3 043 681
- US-A- 4 541 868
- US-A- 5 514 331
- FATHI HABASHI: "HANDBOOK OF EXTRACTIVE METALLURGY", 1 January 1997 (1997-01-01), WILEY-VCH, FEDERAL REPUBLIC OF GERMANY, XP002712891, ISBN: 3-527-28792-2 vol. I, II * page 454, paragraph 7.6.1 - page 457; figure 7.28 * * page 439, paragraph 7.5.2 - page 448, paragraph 7.5.3.3; figures 7.20, 7.21, 7.24 * * page 767 - page 770; figure 12.21 *

## Description

The invention relates to a method for manufacturing an austenitic stainless steel, more particularly to a method for manufacturing an austenitic stainless steel from a nickel laterite ore and a chromite ore.

In a conventional method for manufacturing an austenitic stainless steel, scrap and ferroalloy are used as main raw materials and are smelted into a molten metal in an electric furnace. The molten metal is then transferred to a converter along with adding a ferronickel and/or a ferrochrome into the converter in a ratio determined according to the specific steel to be made (for example, 200 or 300 series stainless steel), thereby obtaining an austenitic stainless steel. Since the cost for a noble metal such as nickel is about 40-50% of the total cost for the stainless steel, the profit of the stainless steel manufacturer is easily affected or even lost due to the price volatility of the noble metal.

There has been developed a process for producing a stainless steel master alloy by directly smelting a nickel laterite ore and a chromite ore as raw materials in an electric furnace or a blast furnace, as disclosed in Chinese Patent Publication Nos. CN 102212691A and CN 101701312A, so as to save the cost for manufacturing a stainless steel. However, in the process disclosed in the aforesaid prior art, the nickel laterite ore and the chromite ore are not pretreated to remove free water and crystallization water prior to the smelting procedure, and a relatively great amount of energy is consumed to remove water during the smelting procedure. Prior art document DE102007050478 discloses the production of stainless steel by alloying elements chromium and nickel, wherein the required intermediate production of ferrochrome and ferronickel takes place in parallel in two separate direct reduction processes on the basis of inexpensive chromium ore and nickel ore.

Furthermore, there are other disadvantages in the process of the aforesaid prior art, such as difficulty in control of the nickel content in the molten metal, relatively great amount of impurities, and inferior recovery rate. Additionally, rare metal such as cobalt usually contained in the nickel laterite ore cannot be extracted and recovered in the process of the aforesaid prior art.

Therefore, the object of the present invention is to provide a cost-effective method for manufacturing an austenitic stainless steel from a nickel laterite ore and a chromite ore.

According to an example not according to this invention, there is provided a method for manufacturing an austenitic stainless steel from a nickel laterite ore and a chromite ore. The method includes steps of:
a) crushing, screening, and blending the nickel laterite ore, followed by roasting the nickel laterite ore in a rotary kiln to remove free water and crystallization water along with charging a reducing agent into the rotary kiln to obtain a calcine, and smelting the calcine in an electric furnace to obtain a molten ferronickel;
b) sintering the chromite ore in a sintering device to obtain a sintered chromite ore, followed by smelting the sintered chromite ore along with a coke particle in another electric furnace to obtain a molten ferrochrome;
c) hot charging the molten ferronickel and the molten ferrochrome into a converter to obtain a molten stainless steel; and
d) charging the molten stainless steel into a continuous casting machine to obtain a stainless steel slab.

According to a second example not according to this invention, there is provided a method for manufacturing an austenitic stainless steel from a nickel laterite ore and a chromite ore. The method includes steps of:
a) crushing the nickel laterite ore and pulping the nickel laterite ore with water to form a pulp material, followed by agitating the pulp material with a sulfuric acid solution under a high pressure atmosphere to form a mixture, filtering a leach solution containing nickel and cobalt out of the mixture, separating the leach solution by solvent extraction into an extraction solution containing nickel and an anti-extraction solution containing cobalt, and electrolyzing the extraction solution and the anti-extraction solution to obtain pure nickel and pure cobalt, respectively;
b) sintering the chromite ore in a sintering device to obtain a sintered chromite ore, followed by smelting the sintered chromite ore in an electric furnace to obtain a molten ferrochrome;
c) transferring the pure nickel into a converter, and hot charging the molten ferrochrome into the converter to obtain a molten stainless steel; and
d) charging the molten stainless steel into a continuous casting machine to obtain a stainless steel slab.

According to an embodiment of this invention, there is provided a method for manufacturing an austenitic stainless steel from a nickel laterite ore and a chromite ore according to Claim 1. The method includes steps of:
a) determining whether a nickel content of the nickel laterite ore is less than 1.5 wt% based on total weight of the nickel laterite ore;
b) processing the nickel laterite ore into a nickel-containing precursor based on the determination made in step a);
c) sintering the chromite ore in a sintering device to obtain a sintered chromite ore, followed by smelting the sintered chromite ore along with a coke particle in an electric furnace to obtain a molten ferrochrome;
d) transferring the nickel-containing precursor into a converter, and hot charging the molten ferrochrome into the converter to obtain a molten stainless steel;
   and
e) charging the molten stainless steel into a continuous casting machine to obtain a stainless steel slab.

A method for manufacturing an austenitic stainless steel from a nickel laterite ore and a chromite ore according to a first example not according to the invention includes steps of:
i) obtaining a molten ferronickel:
   The nickel laterite ore is dried in a drying kiln at a drying temperature ranging from 600 °C to 700 °C to remove free water contained in the nickel laterite ore from 30-35% to 10-20%. The nickel laterite ore is then crushed, screened, and blended, followed by roasting in a rotary kiln at a roasting temperature ranging from 800 °C to 950 °C to remove residual free water and crystallization water from the nickel laterite ore. When the nickel laterite ore is roasted in the rotary kiln, a reducing agent such as anthracite coal is fed into the rotary kiln to obtain a pre-reduced calcine.
   The calcine is molten in an electric furnace to obtain the molten ferronickel. The tapping temperature of the slag is controlled in a range from 1550 °C to 1650 °C and the tapping temperature of the molten ferronickel is controlled in a range from 1400 °C to 1500 °C so as to obtain a better effect for separating the slag from the molten ferronickel. The molten ferronickel includes:
   8-15 wt% of Ni, less than 4 wt% of C, less than 2 wt% of Si, and less than 0.06 wt% of P.
ii) obtaining a molten ferrochrome:
   The chromite ore (content of Cr2O3: less than 62 wt%) is mixed with a coke powder and is pressed in a ball press machine to form chromite pellets, followed by drying the chromite pellets to remove water. The dried chromite pellets are then sintered in a sintering device at a temperature ranging from 1350 °C to 1450 °C to obtain a sintered chromite ore having a particle size less than 30 mm. The sintered chromite ore along with a coke particle is then molten in another electric furnace to obtain the molten ferrochrome. The tapping temperature of the slag is controlled in a range from 1600 °C to 1700 °C. The molten ferrochrome includes: less than 60 wt% of Cr, less than 9 wt% of C, less than 5 wt% of Si, and less than 0.03 wt% of P.
iii) obtaining a molten stainless steel: The molten ferronickel and the molten ferrochrome are transferred into a converter in a hot charging manner to obtain the molten stainless steel.
iv) obtaining a stainless steel slab:
   The molten stainless steel is charged into a continuous casting machine to obtain the stainless steel slab.
   The aforesaid steps iii) and iv) can be conducted in a manner well known in the art, and thus are not described in detail herein.

The molten ferronickel and the molten ferrochrome can be added into the converter in a ratio determined according to the specific stainless steel to be manufactured. For example, the 202 series stainless steel contains 4-6 wt% of Ni and 17-19 wt% of Cr, and the 304 series stainless steel contains 8-10.5 wt% of Ni and 17.5-19.5 wt% of Cr. When the molten ferronickel obtained in step i) contains 8 wt% of Ni, and the molten ferrochrome obtained in step ii) contains 50 wt% of Cr, the 202 series stainless steel can be manufactured by formulating 65 wt% of the molten ferronickel with 35 wt% of the molten ferrochrome. When the molten ferronickel obtained in step i) contains 15 wt% of Ni, and the molten ferrochrome obtained in step ii) contains 40 wt% of Cr, the 304 series stainless steel can be manufactured by formulating 55 wt% of the molten ferronickel with 45 wt% of the molten ferrochrome.

In the aforesaid example not according to the invention, the molten ferronickel and the molten ferrochrome are obtained respectively from the nickel laterite ore and the chromite ore, the stainless steel of various series can be manufactured by formulating the molten ferronickel with the molten ferrochrome in a specific ratio of the molten ferronickel to the molten ferrochrome, which can be easily adjusted and controlled according to the specific stainless steel to be manufactured. Therefore,
the consumption of fuel and electricity can be reduced due to the reduction of the repeated melting times, and the manufacturing cost can be effectively controlled so as to raise the profit for the manufacturer.

A method for manufacturing an austenitic stainless steel from a nickel laterite ore and a chromite ore according to a second example not according to the invention includes steps of:
I) obtaining pure nickel and pure cobalt:
   The nickel laterite ore is crushed and pulped with water to form a pulp material, followed by agitating the pulp material with a sulfuric acid solution under a high pressure atmosphere to form a mixture. A solid-liquid ratio of the nickel laterite ore to the sulfuric acid solution is about 1:4 in the mixture. The pulp material is agitated with the sulfuric acid solution under a pressure ranging from 4 to 5 MPa and at a temperature ranging from 250 °C to 300°C. A leach solution containing nickel and cobalt is then filtered out of the mixture. The leach solution is separated by solvent extraction into an extraction solution containing nickel and an anti-extraction solution containing cobalt. The extraction solution and the anti-extraction solution are electrolyzed to obtain pure nickel and pure cobalt, respectively. The purity of the pure nickel is greater than 99 wt%, and the recovery rate of the pure nickel and cobalt is greater than 90% in the example not according to the invention.
II) obtaining a molten ferrochrome:
   This step can be conducted in a manner identical to the aforesaid step ii) in the first example not according to the invention.
III) obtaining a molten stainless steel:
   The pure nickel is transferred into a convertor via a belt conveyor, and the molten ferrochrome is hot charged into the convertor to obtain the molten stainless steel.
IV) obtaining a stainless steel slab:
   This step can be conducted in a manner identical to the aforesaid step iv) in the first example not according to the invention.

When the pure nickel obtained in step I) has a purity of 99 wt%, and the molten ferrochrome obtained in step II) contains 24 wt% of Cr, the aforesaid 202 series stainless steel can be manufactured by formulating 5 wt% of the pure nickel, 75 wt% of the molten ferrochrome, and 20 wt% of a carbon steel scrap. The aforesaid 304 series stainless steel can be manufactured by formulating 9 wt% of the pure nickel, 76 wt% of the molten ferrochrome, and 15 wt% of a carbon steel scrap.

In addition to the aforesaid effect achievable in the first example not according to the invention, in which the stainless steel of various series can be manufactured by formulating the pure nickel, the molten ferrochrome, and the carbon steel scrap in a specific ratio thereof, valuable pure cobalt can be obtained in the aforesaid step I) along with the pure nickel so as to obtain an additional economic benefit.

A method for manufacturing an austenitic stainless steel from a nickel laterite ore and a chromite ore according to an embodiment of the present invention includes steps of:
A) determining a nickel content of a nickel laterite ore:
   When the nickel content of the nickel laterite ore is determined to be not less than 1.5 wt% based on total weight of the nickel laterite ore, the following steps are performed.
B) obtaining a molten ferronickel:
   This step can be conducted in a manner identical to the aforesaid step i) in the first example not according to the invention.
C) obtaining a molten ferrochrome:
   This step can be conducted in a manner identical to the aforesaid step ii) in the first example not according to the invention.
D) obtaining a molten stainless steel: This step can be conducted in a manner identical to the aforesaid step iii) in the first example not according to the invention.
E) obtaining a stainless steel slab:
   This step can be conducted in a manner identical to the aforesaid step iv) in the first example not according to the invention.

As described above, the molten ferronickel and the molten ferrochrome can be added into the converter in a ratio determined according to the specific stainless steel to be manufactured.

On the other hand, when the nickel content of the nickel laterite ore is determined to be less than 1.5 wt% based on total weight of the nickel laterite ore, the following steps are performed.

### B') obtaining pure nickel and pure cobalt:

This step can be conducted in a manner identical to the aforesaid step I) in the second example not according to the invention.

### C') obtaining a molten ferrochrome:

This step can be conducted in a manner identical to the aforesaid step ii) in the first example not according to the invention.

### D') obtaining a molten stainless steel:

This step can be conducted in a manner identical to the aforesaid step III) in the second example not according to the invention.

### E') obtaining a stainless steel slab:

This step can be conducted in a manner identical to the aforesaid step IV) in the second example not according to the invention.

As described above, the stainless steel of various series can be manufactured by formulating the pure nickel with the molten ferrochrome along with the carbon steel scrap in a specific ratio, which can be easily adjusted and controlled according to the specific stainless steel to be manufactured. Furthermore, other noble metals, such as pure cobalt, can be obtained along with the pure nickel in the electrolytic step. Therefore, the economic value of the method for manufacturing an austenitic stainless steel of the present invention can be further raised.

Alternatively, in the embodiment, both the molten ferronickel and the pure nickel can be transferred into the convertor, and the molten ferrochrome is hot charged into the convertor so as to obtain the molten stainless steel.

In the method for manufacturing an austenitic stainless steel of the present invention, the nickel laterite ore can be effectively treated to obtain a molten ferronickel or a pure nickel. Therefore, the method for manufacturing an austenitic stainless steel of the present invention is relatively flexible and cost-effective as compared to the prior art.

## Claims

1. A method for manufacturing an austenitic stainless steel from a nickel laterite ore and a chromite ore, said method being **characterized by** steps of:
a) determining whether a nickel content of the nickel laterite ore is less than 1.5 wt% based on total weight of the nickel laterite ore;
b) processing the nickel laterite ore into a nickel-containing precursor based on the determination made in step a), wherein the nickel-containing precursor comprises a molten ferronickel or a pure nickel or a combination thereof, and **characterized in that**,
when the nickel content of the nickel laterite ore is determined to be not less than 1.5 wt%, the nickel-containing precursor is a molten ferronickel, and step b) is conducted by crushing, screening, and blending the nickel laterite ore, followed by roasting the nickel laterite ore in a rotary kiln to remove free water and crystallization water along with charging a reducing agent into the rotary kiln to obtain a calcine, and smelting the calcine in another electric furnace to obtain the molten ferronickel;
when the nickel content of the nickel laterite ore is determined to be less than 1.5 wt%, the nickel-containing precursor is pure nickel, and step b) is conducted by crushing the nickel laterite ore and pulping the nickel laterite ore with water to form a pulp material, followed by agitating the pulp material with a sulfuric acid solution under a high pressure atmosphere to form a mixture, filtering a leach solution containing nickel and cobalt out of the mixture, separating the leach solution by solvent extraction into an extraction solution containing nickel and an anti-extraction solution containing cobalt, and electrolyzing the extraction solution and the anti-extraction solution to obtain pure nickel and pure cobalt, respectively;
c) sintering the chromite ore in a sintering device to obtain a sintered chromite ore, followed by smelting the sintered chromite ore along with a coke particle in an electric furnace to obtain a molten ferrochrome;
d) transferring the nickel-containing precursor into a converter, and hot charging the molten ferrochrome into the converter to obtain a molten stainless steel, the nickel-containing precursor transferred into the converter including the molten ferronickel and the pure nickel; and
e) charging the molten stainless steel into a continuous casting machine to obtain a stainless steel slab.

2. The method for manufacturing an austenitic stainless steel as claimed in Claim 1, **characterized in that** in step b), a roasting temperature of the rotary kiln ranges from 800°C to 950°C and a tapping temperature of the molten ferronickel ranges from 1400°C to 1500°C.

3. The method for manufacturing an austenitic stainless steel as claimed in Claim 1, further **characterized by** a step of drying the nickel laterite ore in a drying kiln to remove a portion of the free water prior to step b) .

4. The method for manufacturing an austenitic stainless steel as claimed in Claim 1, **characterized in that** in step b), a solid-liquid ratio of the nickel laterite ore to the sulfuric acid solution is about 1:4, and the pulp material is agitated with the sulfuric acid solution under a pressure ranging from 4 to 5 MPa and at a temperature ranging from 250°C to 300°C.

5. The method for manufacturing an austenitic stainless steel as claimed in Claim 1, further **characterized by** steps of pressing the chromite ore with a coke powder in a ball press machine to form chromite pellets and drying the chromite pellets to remove water prior to step c).

6. The method for manufacturing an austenitic stainless steel as claimed in Claim 1, **characterized in that** in step c), the sintered chromite ore has a particle size less than 30 mm.

## Patentansprüche

1. Verfahren zum Herstellen eines austenitischen rostfreien Stahls aus einem Nickel-Laterit-Erz und einem Chromit-Erz, wobei das Verfahren **gekennzeichnet ist durch** die Schritte:
a) Bestimmen, ob ein Nickelgehalt des Nickel-Laterit-Erzes bezogen auf das Gesamtgewicht des Nickel-Laterit-Erzes weniger als 1,5 Gew.-% beträgt;
b) Verarbeiten des Nickel-Laterit-Erzes basierend auf der in Schritt a) ausgeführten Bestimmung zu einem Nickel enthaltenden Vorläufer, wobei der Nickel enthaltende Vorläufer schmelzflüssiges Ferronickel oder ein reines Nickel oder eine Kombination davon umfasst, und **dadurch** gekennzeichnet umfasst, dass,
wenn bestimmt wird, dass der Nickelgehalt des Nickel-Laterit-Erzes nicht weniger beträgt als 1,5 Gew.-%, der Nickel enthaltende Vorläufer ein schmelzflüssiges Ferronickel ist und Schritt b) ausgeführt wird **durch** Zerkleinern, Sieben und Mischen des Nickel-Laterit-Erzes, gefolgt von einem Rösten des Nickel-Laterit-Erzes in einem Drehrohrofen, um freies Wasser und Kristallisationswasser zu entfernen, zusammen mit dem Einbringen eines reduzierendes Mittels in den Drehrohrofen, um ein geröstetes Produkt zu erhalten, und Schmelzen des gerösteten Produkts in einem anderen elektrischen Ofen, um das schmelzflüssige Ferronickel zu erhalten;
wenn bestimmt wird, dass der Nickelgehalt des Nickel-Laterit-Erzes weniger beträgt als 1,5 Gew.-%, der Nickel enthaltende Vorläufer reines Nickel ist, und Schritt b) ausgeführt wird **durch** Zerkleinern des Nickel-Laterit-Erzes und Aufschließen des Nickel-Laterit-Erzes mit Wasser, um ein Aufschlussmaterial zu bilden, gefolgt von Rühren des Aufschlussmaterials in einer Hochdruckatmosphäre, um eine Mischung zu bilden, Abfiltrieren einer Nickel und Cobalt enthaltenden Laugenslösung aus der Mischung, Auftrennen der Laugenslösung **durch** Lösemittelextraktion zu einer Extraktionslösung, die Nickel enthält, und einer Anti-Extraktionslösung, die Cobalt enthält, sowie Elektrolysieren der Extraktionslösung und der Anti-Extraktionslösung, um reines Nickel bzw. Cobalt zu erhalten;
c) Sintern des Chromit-Erzes in einer Vorrichtung zum Sintern, um ein gesintertes Chromit-Erz zu erhalten, gefolgt **durch** Schmelzen des gesinterten Chromit-Erzes zusammen mit einem Koksteilchen in einem elektrischen Ofen, um ein schmelzflüssiges Ferrochrom zu erhalten;
d) Überführen des Nickel enthaltenden Vorläufers in einen Konverter und heißes Einbringen des schmelzflüssigen Ferrochroms in den Konverter, um einen schmelzflüssigen rostfreien Stahl zu erhalten, wobei der in den Konverter überführte Nickel enthaltende Vorläufer das schmelzflüssige Ferronickel und das reine Nickel einschließt; und
e) Einbringen des schmelzflüssigen rostfreien Stahls in eine Maschine zum Stranggießen, um eine Bramme aus rostfreiem Stahl zu erhalten.

2. Verfahren zum Herstellen eines austenitischen rostfreien Stahls nach Anspruch 1, **dadurch gekennzeichnet, dass** in Schritt b) eine Rösttemperatur des Drehrohrofens im Bereich von 800 °C bis 950 °C liegt und eine Abstichtemperatur des schmelzflüssigen Ferronickels im Bereich von 1.400 °C bis 1.500 °C liegt.

3. Verfahren zum Herstellen eines austenitischen rostfreien Stahls nach Anspruch 1, ferner **gekennzeichnet durch** einen Schritt des Trocknens des Nickel-Laterit-Erzes in einem Trockenofen, um einen Teil des freien Wassers vor dem Schritt b) zu entfernen.

4. Verfahren zum Herstellen eines austenitischen rostfreien Stahls nach Anspruch 1, **dadurch gekennzeichnet, dass** in Schritt b) ein Fest-Flüssig-Verhältnis des Nickel-Laterit-Erzes zu der Schwefelsäurelösung etwa 1: 4 beträgt und das Aufschlussmaterial mit der Schwefelsäurelösung unter einem Druck im Bereich von 4 bis 5 MPa und bei einer Temperatur im Bereich von 250 °C bis 300 °C gerührt wird.

5. Verfahren zum Herstellen eines austenitischen rostfreien Stahls nach Anspruch 1, ferner **gekennzeichnet durch** Schritte des Pressens des Chromit-Erzes mit einem Kokspulver in einer Kugelpressmaschine zur Bildung von Chromit-Pellets und Trocknen der Chromit-Pellets zur Entfernung von Wasser vor Schritt c).

6. Verfahren zum Herstellen eines austenitischen rostfreien Stahls nach Anspruch 1, **dadurch gekennzeichnet, dass** in Schritt c) das gesinterte Chromit-Erz eine Partikelgröße kleiner als 30 mm aufweist.

## Revendications

1. Procédé pour la fabrication d'un acier inoxydable austénitique à partir d'un minerai de latérite de nickel et d'un minerai de chromite, ledit procédé étant **caractérisé par** les étapes de:
a) détermination si la teneur en nickel du minerai de latérite de nickel est inférieure à 1,5% en poids sur la base du poids total du minerai de latérite de nickel;
b) transformation du minerai de latérite de nickel en un précurseur contenant du nickel sur la base de la détermination faite dans l'étape a), où le précurseur contenant du nickel comprend un ferronickel fondu ou un nickel pur ou une combinaison de ceux-ci, et **caractérisé en ce que**:
lorsqu'il est déterminé que la teneur en nickel du minerai de latérite de nickel n'est pas inférieure à 1,5% en poids, le précurseur contenant du nickel est un ferronickel fondu et l'étape b) est effectuée par un concassage, un tamisage et un malaxage du minerai de latérite de nickel, suivi par un grillage du minerai de latérite de nickel dans un four rotatif pour retirer l'eau libre et l'eau de cristallisation accompagné du chargement d'un agent réducteur dans le four rotatif pour obtenir un produit calciné, et une fusion du produit calciné dans un autre four électrique pour obtenir le ferronickel fondu;
lorsqu'il est déterminé que la teneur en nickel du minerai de latérite de nickel est inférieure à 1,5% en poids, le précurseur contenant du nickel est un nickel pur et l'étape b) est effectuée par un concassage du minerai de latérite de nickel et un pulpage du minerai de latérite de nickel avec de l'eau pour former un matériau de pulpe, suivi par une agitation du matériau de pulpe avec une solution d'acide sulfurique sous une atmosphère haute pression pour former un mélange, une filtration d'une solution de lixiviation contenant du nickel et du cobalt à partir du mélange, une séparation de la solution de lixiviation par une extraction au solvant en une solution d'extraction contenant du nickel et une solution d'anti-extraction contenant du cobalt, et une électrolyse de la solution d'extraction et de la solution d'anti-extraction pour obtenir du nickel pur et du cobalt pur, respectivement;
c) frittage du minerai de chromite dans un dispositif de frittage pour obtenir un minerai de chromite fritté, suivi par une fusion du minerai de chromite fritté accompagné de particules de coke dans un four électrique pour obtenir un ferrochrome fondu;
d) transfert du précurseur contenant du nickel dans un convertisseur et chargement à chaud du ferrochrome fondu dans le convertisseur pour obtenir un acier inoxydable fondu, le précurseur contenant du nickel transféré dans le convertisseur incluant le ferronickel fondu et le nickel pur; et
e) chargement de l'acier inoxydable fondu dans une machine à coulée continue pour obtenir une dalle d'acier inoxydable.

2. Procédé pour la fabrication d'un acier inoxydable austénitique selon la revendication 1, **caractérisé en ce que** dans l'étape b), la température de grillage du four rotatif varie de 800°C à 950°C et la température de coulée du ferronickel fondu varie de 1400°C à 1500°C.

3. Procédé pour la fabrication d'un acier inoxydable austénitique selon la revendication 1, **caractérisé en outre par** une étape de séchage du minerai de latérite de nickel dans un séchoir pour retirer une portion de l'eau libre avant l'étape b).

4. Procédé pour la fabrication d'un acier inoxydable austénitique selon la revendication 1, **caractérisé en ce que** dans l'étape b), le rapport solide-liquide du minerai de latérite de nickel sur la solution d'acide sulfurique est d'environ 1:4 et le matériau de pulpe est agité avec la solution d'acide sulfurique sous une pression variant de 4 à 5 MPa et à une température variant de 250°C à 300°C.

5. Procédé pour la fabrication d'un acier inoxydable austénitique selon la revendication 1, **caractérisé en outre par** des étapes de pressage du minerai de chromite avec une poudre de coke dans une machine presse à boulets pour former des boulettes de chromite et de séchage des boulettes de chromite pour retirer l'eau avant l'étape c).

6. Procédé pour la fabrication d'un acier inoxydable austénitique selon la revendication 1, **caractérisé en ce que** dans l'étape c), le minerai de chromite fritté a une taille de particules inférieure à 30 mm.
